

G. J. MANSON,  
METHOD OF MANUFACTURING FIBER PRODUCTS,  
APPLICATION FILED MAR. 15, 1919.

1,399,976.

Patented Dec. 13, 1921.

2 SHEETS—SHEET 1.



INVENTOR  
GEORGE J. MANSION

BY K.P. McElroy  
ATT Y'LL

1,399,976.

G. J. MANSON.

METHOD OF MANUFACTURING FIBER PRODUCTS.

APPLICATION FILED MAR. 15, 1919.

Patented Dec. 13, 1921.

2 SHEETS—SHEET 2.



INVENTOR  
GEORGE J. MANSON

BY

K. R. McElroy,  
ATTY'S.

# UNITED STATES PATENT OFFICE.

GEORGE JAMES MANSON, OF TORONTO, ONTARIO, CANADA.

## METHOD OF MANUFACTURING FIBER PRODUCTS.

1,399,976.

Specification of Letters Patent. Patented Dec. 13, 1921.

Continuation of application Serial No. 32,418, filed June 5, 1915. This application filed March 15, 1919. Serial No. 282,780.

*To all whom it may concern:*

Be it known that I, GEORGE JAMES MANSON, a subject of the King of Great Britain, and resident of the city of Toronto, in the Province of Ontario, Dominion of Canada, have invented certain new and useful Improvements in Methods of Manufacturing Fiber Products, of which the following is a specification.

10 This invention relates to improvements in methods of manufacturing fiber products, and it consists of a method of making uncooked or chemically untreated, loose, relatively long fibers from raw wood, together with a certain proportion of short fibers, such fibers being adapted to felt or mat together under pressure to form pulp articles or sheets. The process is designed to make use of what is now generally considered a waste material, namely, saw mill waste comprising slabs, edgings, short butting blocks, slats, burner refuse, sawdust, bark and shavings; and one of the advantages of the process is that by the use of this material in 25 the manner hereinafter set forth it is possible to obtain a better fiber board than can be obtained if ordinary pulp wood were ground up. In carrying out the process the saw mill waste is first chipped; it is then fed with water between the grinding surfaces of spaced grinding elements set a short distance apart and having relative movement to each other, being passed between such surfaces for a sufficient length of time to reduce it to 30 a flexible, feltable fibrous material directly adaptable for the manufacture of pulp board; all as more fully hereinafter set forth and described.

In the art, paper pulp is produced mechanically by grinding relatively large blocks of pulp wood, presented to the grinding face side on, under high pressure, which gives a relatively short fiber. Paper pulp has also been manufactured from chips 40 which are chemically digested in one way or another, or softened in water and then passed through a grinder or like fiber-treating machine. This treatment has the effect of removing or softening the barbs on the fibers thereby impairing the capacity for felting.

In the invention of the present application, which is a continuation of my earlier application Serial No. 32,418 filed June 5, 55 1915, I operate in a different manner and

produce a relatively large proportion of long fibered material together with a certain quantity of short fibered material which assists in filling in the spaces between the longer fiber and also interlocks therewith. 60

In practising the process I first comminute the raw wood by the use of an ordinary chipper to which it is fed by gravity and which produces chips of a size from five-eighths to three-quarters of an inch with the grain, and 65 one-eighth to one-quarter of an inch across the grain. The wood is preferably in the form of saw mill waste including slabs, edgings, short butting blocks, slats, burner refuse, sawdust, bark and shavings. No water 70 is added to the wood, as it ordinarily will be found to contain from forty-five to sixty per cent. of water, but this may be as low as twenty-five per cent. if the material has been standing some time. 75

The raw wood so comminuted is then passed between tapering grinding surfaces having but a narrow clearance between them, the clearance however being sufficiently wide to accommodate a plurality of 80 fibers side by side. Through this passage-way the comminuted wood is transmitted with a small stream of water, the proportion of water being such that the material coming from the grinder contains about eighty 85 to ninety per cent. of water. The material is passed through the grinder in such a way that there is a continuous film of comminuted raw wood between the moving grinding surfaces, the operation being conducted in such a manner as to cause the action to be more that of the fibers rubbing against each other than that of rubbing directly against the grinding surfaces. From 90 which it results that relatively long fiber 95 bundles are produced, many of the fibers coming through in bundles with their ends free to interlock with other fibers when pressed.

The grinding surfaces between which the 100 comminuted wood is passed are not, in the present invention really the comminuting means, their roughened surfaces being used more for the purposes of friction, to cause positive movement of the fibers. More reliance is placed on the mutual rubbing action of the wood particles on each other for producing the lateral separation of the fibrous elements from each other. Since the 105 wood is comminuted before its entry be- 110

tween these surfaces, the fibers are not broken off short, as is inevitable when the wood is presented to a grinding surface under great pressure. In a way, my operation is more what may be termed a rolling separation of the fibers than a true grinding action.

The purpose of adding the water to the mixture before passing into the grinder is to 10 keep down the temperature and at the same time to make the mass fluid enough so that it will feed through the grinders.

The wood is not steamed, soaked in water, treated with chemicals or otherwise chemically 15 prepared in any way prior to my fiber making operation, it is raw wood which I use, wood which has not been changed otherwise than by the necessary comminution. The material or stock coming 20 from between the grinding surfaces is then screened in a standard centrifugal or flat screen. Where the centrifugal screen is used I prefer to employ a "ninety" plate, that is to say, a plate with holes .090 inches 25 in diameter, the tailings from which screen are returned to the grinder. Before screening, sufficient water is added to render the stock quite fluid, that is to say, until there are about three hundred parts water to one 30 part stock. The fiber product coming from the screens may be used in same manner as other pulp fiber products, are used in the trade. I prefer to continue the process to make a pulp brand as hereinafter described. 35 After being screened the stock is thickened. The water added before screening is removed by passing through any standard thickener. The stock is left with about ninety-seven parts water, or a three per cent. 40 mixture.

This three per cent. mixture of pulp and water is then run through a press, which may be of any convenient type depending upon the article to be produced. When 45 pulp sheets are to be pressed I employ from three hundred to three hundred and fifty pounds per square inch pressure and press the stock from about six inches depth in the die to about nine-sixteenths of an inch. 50 Thus the final fiber board produced contains about fifty per cent. of pulp and fifty per cent. of water.

This fiber board is then dried practically 55 bone dry in a suitable dryer, its edges trimmed to size and the surface may be finished by water proofing. It will be found desirable by means of waterproofing or other means to add about seven per cent. of water to the bone dry board in order to produce a 60 board which will have a water contents corresponding with that of the atmosphere.

It will be found that the fiber product produced by the process described has special qualities in that there are a relatively 65 large percentage of long fiber bundles, by

which is meant one-quarter to three-quarters of an inch in length, and that these fiber bundles are thoroughly barbed and adapted to interlock. With these long fiber bundles there is a certain percentage of short fibers 70 or fiber bundles resulting from the sawdust and other short chips of wood and these are useful to fill in the voids and to interlock with the longer fibers. The amount of sawdust in the raw material is preferably such 75 that the product will have from twenty-two to twenty-eight per cent. of short fibers. It will be found also that the long fibers will not be completely separated from each other but will be present in bundles having 80 their ends free to interlock; which ends are thoroughly barbed, because the rolling action in the grinder of the fibers, one against the other, still leaves the fiber raw and in bundles and with the barbs thereon 85 produced by the loosened or brushed out ends of the individual fibers.

The fiber board made from ground wood pulp will be found much denser than board produced from the fibers produced according to my process as the fibers are smoother than that produced by my process, but this dense board has not as high an insulating value and is not as economical to manufacture. The board produced from the fibers 90 produced in my process will be found to have a slight brownish tinge owing to the presence of the bark. The gums and resin in the bark will also cause a closer adhesion of the fibers acting more or less, as binding 95 means.

The grinding surface referred to in the foregoing process may be of a variety of forms, I have devised, however, a form of grinder in which the process may be economically carried out and which is shown in the drawings accompanying this specification. 105

In the drawings:

Figure 1 is a sectional elevation of the 110 apparatus.

Fig. 2 is a plan view of the adjusting mechanism.

Fig. 3 is a side view of the rotating grinding element.

Fig. 4 is an end view of the grinding element.

Fig. 5 is a view of a bundle of the barbed fiber of raw wood produced for use in the manufacture of the fiber board according to 120 the present method.

Fig. 6 is a view showing the ordinary fiber of ground wood pulp.

In the drawings like characters of reference indicate corresponding parts in all the 125 figures.

Referring to the drawings, A represents a suitable base having standards 10, 11 and 12 which support the shaft B adapted to be turned by a convenient source of power 130

conveniently applied to the shaft through the pulley 13.

Means are provided for adjusting the shaft in an axial direction. The well known means which I show to accomplish this purpose comprise a hand wheel 14 adapted to turn a pinion 15 which meshes with gears 16 and 17 connected to screw shafts 18 and 19 which extends through a traveling element 20 which has a collar 21 fitting between the collars 22 and 23 on the shaft B. Ball bearings 24 are shown between the collar 21 and the collars 22 and 23. Any other convenient and well known means for adjusting the shaft in a lengthwise direction may be employed.

C represents the rotary grinding element which is conical in form, the outer surface being substantially at an angle of 30° to the axis. This element is secured to and rotates with the shaft B and is adapted to co-operate with the fixed element D of the grinding pair which is secured to the fixed casing E. Material is adapted to be fed between the grinding element from a feeding chamber 30 at the small end of said members and the ground fibers are adapted to be withdrawn from the larger peripheries of the grinding pair from the outlet box 31. The feeding may be facilitated by a worm conveyer 32 mounted on the shaft B within the feeding chamber 30.

The grinding element may be of sandstone or an artificial sandstone such as is manufactured from a mixture of cement and sharp sand in equal proportions with a small percentage, say 10%, of soft material such as sawdust, to produce voids therein.

The rotary grinding element C is provided on its surface with a plurality of feeding grooves 33 which extend in a spiral manner around on the periphery and are gradually decreased in depth from their commencement at the small end of the cone 45 to their end near the large end of the cone. In this way the stock fed in by the channel moving in an axial direction is gradually, by the reduction in depth of the groove, forced out between the grinding elements.

The grinding elements are adjusted relatively to each other so that there will be enough room between the surfaces for the fiber bundles to rub against each other and not to be rubbed directly between the surfaces.

The stock is fed continuously under moderate pressure and is distributed between the grinding surfaces by grooves 33 as already explained. It is necessary that the continuity of the feed should not be interrupted and that a continuous film of stock be maintained between the surfaces.

Where the conical surfaces are of narrow diameter the stock is broken up while a finish is imparted to it at the high speed of the

grinding surface found at the large end of the cone.

The peculiar, well barbed nature of the fiber produced according to the present process may be seen by the illustrations given in Fig. 5 of the drawings. Fig. 5 represents a well barbed fiber bundle produced according to the rolling action in the present process, while Fig. 6, the ordinary fiber ground wood pulp. It is found that the well barbed fiber produced by my process is more advantageous in making the nap on fibers, in that the barbs interlock to a much greater extent, thereby producing a better nap and one not liable to split or peel.

As many changes could be made in the above process and many apparently widely different embodiments of my invention, within the scope of the claims, produced without departing from the spirit or scope thereof, it is intended that all matter contained in the accompanying specification and drawings shall be interpreted as illustrative and not in a limiting sense.

What I claim as my invention is:

1. The herein described process of manufacturing a fiber product which comprises, first chipping saw mill waste, then grinding the raw chipped wood with water between closely spaced surfaces having a movement relative to each other, such surfaces being sufficiently far apart to permit at the narrowest point the presence of a plurality of fiber bundles therebetween, whereby a rolling separation is effected.

2. The herein described process of manufacturing a fiber product which comprises, first chipping raw wood, then grinding the raw chipped wood with water between closely spaced surfaces having a movement relative to each other, such surfaces being sufficiently far apart to permit at the narrowest point the presence of a plurality of fiber bundles therebetween, whereby a rolling separation is effected, then screening the fibrous material, then thickening the stock of the screening operation, and then pressing the fibers.

3. The herein described process of manufacturing a fiber product which comprises, first chipping raw wood, then grinding the raw chipped wood with water between closely spaced surfaces having a movement relative to each other, such surfaces being sufficiently far apart to permit at the narrowest point the presence of a plurality of fiber bundles therebetween, whereby a rolling separation is effected, then screening the fibrous material, then thickening the stock of the screening operation, then pressing the fibers, then drying the pressed material, and then adding a percentage of water to correspond with atmospheric conditions.

4. The herein described process of manufacturing a fiber product which comprises

first chipping raw wood, then grinding the chipped wood with water between closely spaced surfaces having a movement relative to each other, such surfaces being sufficiently far apart to permit at the narrowest point the presence of a plurality of fibers therebetween, whereby a rolling separation is effected.

5. The herein described process of manufacturing a fiber product which comprises 10 grinding relatively small pieces of raw wood with water between closely spaced surfaces having a movement relative to each other, such surfaces being sufficiently far apart 15 to permit at the narrowest point the presence of a plurality of fiber bundles therebetween whereby a rolling separation is effected.

6. The herein described process of manufacturing a fiber product which comprises 20 grinding relatively small pieces of raw wood with water between closely spaced surfaces having a movement relative to each other, such surfaces being sufficiently far apart to permit at the narrowest point the presence 25 of a plurality of fiber bundles therebetween whereby a rolling separation is effected, then pressing the fibers produced by the aforesaid grinding operation to form a fiber product.

In witness whereof I have hereunto set my hand in the presence of a witness.

GEORGE JAMES MANSON.

Witness:

RUSSEL S. SMART.